

May 7, 1963

J. A. M. LE DUC

3,088,886

PROCESS OF ELECTROPOLISHING ZINC

Filed Nov. 3, 1958

5 Sheets-Sheet 1



FIG. 1

FIG. 2

FIG. 3



FIG. 4

FIG. 5

FIG. 6

INVENTOR  
JOSEPH ADRIEN M. LE DUC

BY *Warburton & Cross*

ATTORNEYS

May 7, 1963

J. A. M. LE DUC

3,088,886

PROCESS OF ELECTROPOOLISHING ZINC

Filed Nov. 3, 1958

5 Sheets-Sheet 2



FIG. 7



FIG. 8



FIG. 9



FIG. 10



FIG. 11



FIG. 12

INVENTOR  
JOSEPH ADRIEN M. LE DUC

BY *Warburton & Cross*

ATTORNEYS

May 7, 1963

J. A. M. LE DUC

3,088,886

PROCESS OF ELECTROPOLISHING ZINC

Filed Nov. 3, 1958

5 Sheets-Sheet 3



FIG. 13

FIG. 14

FIG. 15



FIG. 16

FIG. 17

FIG. 18

INVENTOR  
JOSEPH ADRIEN M. LE DUC

BY *Warburton & Cross*  
ATTORNEYS

May 7, 1963

J. A. M. LE DUC

3,088,886

PROCESS OF ELECTROPOLISHING ZINC

Filed Nov. 3, 1958

5 Sheets-Sheet 4



FIG. 19

FIG. 20

FIG. 21



FIG. 22

FIG. 23

FIG. 24

INVENTOR  
JOSEPH ADRIEN M. LE DUC

BY *Warburton & Cross*

ATTORNEYS

May 7, 1963

J. A. M. LE DUC

3,088,886

PROCESS OF ELECTROPOLISHING ZINC

Filed Nov. 3, 1958

5 Sheets-Sheet 5



LEGEND

CURVE      MATERIALS

- A---PLATINUM
- B---CAST IRON
- C---STAINLESS STEEL -HEAT TREATED
- D---STEEL -HEAT TREATED
- E---MAGNETITE (CAST)
- F---STEEL 10/10
- G---STAINLESS STEEL 310
- H---NICKEL-A (BRIGHT)
- I---PURE ZINC SHEET (BRIGHT)
- J---STEEL SHEET PLATED ZINC

INVENTOR

JOSEPH ADRIEN M. LE DUC

BY *Warburton & Cross*

ATTORNEY

## 1

3,088,886

PROCESS OF ELECTROPOLISHING ZINC  
Joseph Adrien M. Le Duc, Painesville, Ohio, assignor to  
Diamond Alkali Company, Cleveland, Ohio, a corpora-  
tion of Delaware

Filed Nov. 3, 1958, Ser. No. 771,507  
15 Claims. (Cl. 204—140.5)

This invention relates to the electropolishing of zinc and zinc alloys and, more particularly, to a process for the anodic polishing of zinc and zinc alloys and to an electrolyte composition for use in such a process.

Zinc and zinc alloys, particularly zinc alloys containing 90% or more zinc, are presently widely used as the base material for making plated articles, particularly chromium plated articles. In such uses, a casting is made of the zinc or zinc alloy, which casting is customarily then trimmed, strapped and buffed, generally in an automatic buffing machine, to smooth the surface and to eliminate, as much as possible, any pits therein. The surface of the casting is then degreased and cleaned, after which it is plated, first with copper, then nickel and finally chromium, to give the finished plated article.

In this procedure, one operation, that of buffing, is done by hand and is the most time-consuming and expensive, often accounting for as much as 50% of the total finishing cost. Additionally, because all metals possess some degree of malleability, mechanical polishing causes deforming and crushing of the crystal structure of the metal near its surface. This deformation and crushing adversely affects the friction and wear properties of the metal, as well as reducing the corrosion resistance and endurance strength of the metal, even after plating.

In order to overcome the structural disadvantages which result from mechanical buffing, as well as to substantially reduce the time and cost of such an operation, and obtain a deburring as well as brightening of the work-piece, it has been proposed to polish zinc and zinc alloy castings electrolytically. In such operations, electrolytes comprising chromic and/or phosphoric acid have generally been used. However, these materials are relatively expensive and hence the electropolishing operation using such electrolyte baths, are not appreciably more economical than mechanical buffing. Alkaline electrolytes have also been used, such as those consisting of an alkali metal hydroxide and cyanide or an alkali metal hydroxide alone. However, the former bath, because of the cyanide contained therein, is potentially dangerous to those working with it and hence not desirable. For this reason, electrolytes consisting essentially of alkali metal hydroxides, alone, are preferred.

In view of this, considerable work has been done to determine the operating conditions under which electropolishing takes place in an alkali metal hydroxide electrolyte. As reported in the Canadian Journal of Chemistry, vol. 31, 1953, pages 422 to 438, zinc and zinc alloy castings may be electropolished in an alkali metal hydroxide electrolyte containing from about 200 to 1400 g./liter of alkali metal hydroxide using a current density of from 163 to about 909 amps./square foot at a temperature from 32 to 194° F. Additionally, it has been found to be desirable to incorporate small quantities of zinc oxide in the electrolyte to minimize pitting of the casting. However, although the above demonstrates the feasibility of

## 2

electropolishing zinc and zinc alloys in an alkali metal hydroxide electrolyte, on a laboratory basis, the described process has not, up to this time been found to be applicable for commercial operations.

5 The primary cause for the unsatisfactory characteristics of this method is that considerable quantities of spongy zinc are deposited on the cathodes of the electropolishing apparatus during its use. This spongy deposit of zinc on the cathode becomes larger as the electropolishing is continued, loosens itself from the cathode, floats on the electrolyte and becomes mixed therewith. This floating spongy mass comes in contact with the anode work, thereby short-circuiting above the solution, in a hydrogen-oxygen atmosphere, often resulting in an explosion.

In an effort to eliminate the formation of this porous zinc deposit, mercury has been added to the electrolyte so as to cause a harder, more adherent zinc deposit to form on the cathode rather than the spongy zinc ordinarily formed. Although, by the use of such expedient, the initial zinc, plated on the cathode, is hard and non-porous, within a short time the deposit again becomes spongy and floats on the electrolyte surface. Similar results are obtained with other additives, such as lead.

An additional cause of unsatisfactory characteristics of this method is that the alkali metal hydroxide electrolyte, as proposed in the above cited Canadian Journal, is subject to an excessive amount of foaming in use, which foaming due to hydrogen evolution and surface tension of the bath, makes polishing of the zinc or zinc alloys extremely difficult.

It has now been found, in the practice of the present invention, that within the broad ranges of operating conditions, for the anodic electropolishing of zinc and zinc alloys in alkali metal hydroxide electrolytes, as disclosed in the above Canadian Journal, considerably narrower ranges occur, wherein the anodic electropolishing of zinc and zinc alloys may be carried out on a commercial scale. Additionally, it has been found, that where a cathode having a surface containing  $Fe_3O_4$  is used, in an electropolishing process carried out within these narrower ranges of operation, there is no formation of spongy zinc plate on the cathode, the zinc remaining in solution in the alkali metal hydroxide electrolyte. Alternatively, an oxidizing agent or compound having available oxygen can be added to the electrolyte to prevent the plating of zinc on the cathode. It has been found, that contrary to the prior beliefs, the inclusion of zinc oxide in the alkali metal hydroxide electrolyte is not essential, and additionally, that certain materials, which will prevent the foaming of the alkali metal hydroxide electrolyte during electropolishing, can be included in the electrolyte, without any detrimental effect thereto.

It is, therefore, an object of the present invention to provide a commercially feasible process for the anodic electropolishing of zinc and zinc alloys.

Another object of this invention is to provide such a process, whereby the electropolishing takes place in an alkali metal hydroxide electrolyte.

60 A further object of this invention is to provide a suitable alkali metal hydroxide electrolyte for use in the above process.

These and other objects will become apparent to those skilled in the art from the description of the invention which follows.

As used in the description of the invention and the claims, the term, "alkali metal hydroxide," is meant to refer to the hydroxides of lithium, sodium, potassium, cesium and rubidium. However, because of its low cost and ready availability, sodium hydroxide is preferred, and for this reason, primary reference will be made herein-after to sodium hydroxide.

Referring now to the drawings, which are attached hereto and made a part hereof, FIGS. I to XXIV are reproduced from actual photographs of cathodes, of various materials made before and after the cathodes were used in the electropolishing of zinc in alkali metal hydroxide solutions.

FIGS. XXV and XXVI are graphs illustrating the electrode potentials for some of these cathode metals.

In a commercially feasible process for anodically electropolishing zinc and zinc alloys, the method of the present invention envisions the following operative conditions, within the broad range of operating conditions disclosed in the prior art. The concentration of the alkali metal hydroxide, preferably sodium hydroxide, electrolyte, should be within the range of about 450 to 900 g./liter, with the preferred range being 572 to 763 g./liter, i.e., about a 40 to 50% aqueous sodium hydroxide solution. The temperature of the electrolyte may be varied within the range of 60 to 220° F., depending upon the concentration of the electrolyte which is used. At the higher electrolyte concentrations, e.g., 800 to 900 g./liter, the preferred temperature range is 125 to 162° F. However, with the preferred electrolyte concentration of 572 to 763 g./liter, these high temperatures will not produce the most effective electropolishing of zinc and zinc alloys, while temperatures within the range of 70 to 90° F. give the best electropolishing and hence are the preferred temperatures for this concentration range.

Within the above ranges of electrolyte compositions, at the preferred temperatures given, satisfactory electropolishing of zinc and zinc alloys is carried out over a wide range of current densities, e.g., 50 to 800 amps./square foot for various periods of time. For example, at the higher current densities, the time required for good electropolishing will be about 1-2 minutes, while at lower current densities, the time required will increase to 4 minutes or somewhat more. However, it will be appreciated by those skilled in the art, because of the higher electrical load carrying equipment which is required to provide high current densities, which equipment is not standard in most electrolytic apparatus, current densities of about 200 amps./square foot are preferred. At this current density about 4 minutes is required for good electropolishing. Additionally, it has been found, that in the electropolishing process carried out under these conditions, the solution current density, which may be defined as the total applied current divided by the total effective volume of electrolyte, should not be in excess of about 2.5 amps./liter. Where this value is exceeded, the zinc or zinc alloy castings are polished but zinc is plated on the cathode.

It has been found, that even when operating the electropolishing process under the above preferred conditions, a spongy, porous zinc is plated on the cathode, which zinc plate, if deposition is permitted to continue, will eventually cause a short circuit in the cell. It has now also been found, that when operating under the above preferred conditions, this zinc deposit is eliminated by using a cathode having a surface which contains  $Fe_3O_4$ . It is to be recognized that  $Fe_3O_4$  is frequently expressed as  $Fe_2O_3 \cdot FeO$  and as such designation is included in the present invention. Examples of such material are heat-treated steel, black oxide coated steel, hot-rolled steel, magnetite and any other metal or non-metal on which there is a surface which contains  $Fe_3O_4$ . Additionally, by a cathode having a surface which contains  $Fe_3O_4$ , it is meant to include cast iron, which has likewise been found to exhibit the same desirable qualities as the materials mentioned above. Preferred among

such cathodes is one of hot-rolled steel or black oxide coated steel. Such a cathode may be in the form of one or several plates or if desired may be the tank which contains the electrolyte. When such a cathode is used, 5 there is no deposition of a spongy, porous zinc plate thereon, the zinc remains in solution as zincate and considerable quantities of hydrogen gas are discharged at the cathode. For the most effective operations, that is, in order to get the most complete dissolution of the zinc 10 into the solution, the area of the cathode should be of the order of 10-40 times the area of the anode.

Alternatively, to prevent a build-up of zinc on the cathode, an oxidizing agent may be added to the electrolyte. Examples of such materials are perborates, peroxydisulfates, oxychlorides, permanganates, bichromates, 15 chlorates, bromates, iodates, nitrates, peroxides, and chlorine. Particularly good results have been obtained using the alkali metal perborates, peroxydisulfates, peroxides and nitrates and the alkaline earth metal oxychlorides, specifically, sodium nitrate, sodium perborate, potassium peroxydisulfate, and sodium peroxide and calcium oxychloride. Although, addition of these materials, in the mount of about 20-25 gms./liter of electrolyte is effective in avoiding plating at the cathode, 20 these agents must be replenished about once every eight hours. Because of this, the preferred method of preventing a build-up of zinc on the cathode is the use of a cathode having a surface which contains  $Fe_3O_4$ .

While the oxidizing agent in the electrolyte avoids 25 plating of zinc at the cathode the exact mechanism by which the  $Fe_3O_4$  containing surface on the cathode prevents zinc plating is not known. It is believed, however, that the hydrogen overvoltage value of the  $Fe_3O_4$  coated cathode has greatly changed the characteristics of the 30 system, so that the current does not plate zinc on the cathode, but rather electrolyzes the contents of the electrolyte, hydrogen being given off at the cathode and the oxygen combining with the zinc and the alkali to form a zincate, which gradually builds up in concentration during 35 electropolishing.

While previously, it was believed to be essential that 40 the alkali metal hydroxide electrolyte, such as sodium hydroxide, contain zinc oxide when the electropolishing begins, in order to prevent pitting of the zinc or zinc alloys which are being polished, it is also known that the 45 addition of zinc oxide to the electrolyte is undesirable, in that as the electropolishing continues, there is a gradual build-up of zinc oxide in the electrolyte until a point is reached at which electropolishing no longer takes place. This point, that is, the concentration of zinc oxide which 50 can be tolerated in the electrolyte, has been found to be about 175 g./liter.

Thus, it can be seen that when zinc oxide is initially 55 added to the electrolyte, the effective electropolishing of the electrolyte, prior to the time replenishment is required, will be shortened. It has now been found, that in a 60 commercial operation, wherein the electropolishing conditions are within the preferred ranges set forth above, although the presence of zinc oxide in the electrolyte does not adversely affect electropolishing, it can likewise be 65 eliminated from the initial bath composition without deleteriously affecting the electropolishing of zinc or zinc alloys, since it accumulates during the electropolishing operation. In actual practice, an electrolyte bath consisting essentially of a 40 to 50% solution of sodium hydroxide may be used for a period of about 2 to 3 weeks before the zinc oxide concentration therein builds-up to the toleration point of 175 g./liter, whereupon the entire 70 bath may be renewed or any portion thereof may be replenished, which is necessary to reduce the zinc oxide concentration to below the toleration point. Alternatively, the bath may be dragged out every day either by removal or loss of solution and the caustic soda electrolyte replenished by the addition of about 5%, by volume of 75 the total bath, caustic soda, thereby maintaining the zinc

oxide concentration in the bath below the toleration point for a period of 6 months or more, after which time the entire bath, generally, will have to be replaced.

Additionally, it has been found to be desirable, although not essential, to add to the above sodium hydroxide electrolyte solution a small amount, e.g., .003-.03% by weight, of a material which acts as a defoaming agent. Examples of materials which may be so used are the following:

Anisole  
Dimethyl octynediol  
Phenol  
Cocoyl surcosine  
Cresol  
Lauric isopropanolamide  
Mono-butyl naphthalene sodium sulfonate  
Di-butyl naphthalene sodium sulfonate  
Nonyl phenoxy polyoxyethylene ethanol  
Disodium-N-octadecylsulfosuccinamate  
Aliphatic substituted butynediols  
Aliphatic substituted octynediols  
Aliphatic substituted octynediols mixed with an alkyl phenyl ether of polyethylene glycol in ethylene glycol  
Alkyl benzyl polyethylene glycol ether  
Polyoxyethylene esters of mixed fatty and rosin acids  
Polyethylene tridecyl alcohol  
Polyethylene tridecyl alcohol and urea  
Branched chain alcohol ethers  
Alkyl phenyl polyethylene glycol ether  
Polyalkylene glycol ethers  
Polyoxyethylene ester  
Compounds formed by addition of propylene oxide to ethylene-diamine followed by addition of ethylene oxide

Of these, cresol, aliphatic substituted octynediols, aliphatic substituted octynediols mixed with an alkyl phenyl ether of polyethylene glycol in ethylene glycol, alkyl benzyl polyethylene glycol ether and polyoxyethylene esters of mixed fatty and rosin acids are preferred.

Where the caustic electrolyte solution is used without a defoaming agent, there is a considerable frothing and foam formation in the electrolyte, which foam, by adhering to the anode and cathode, makes electropolishing of the work pieces extremely difficult. It will be appreciated that this foam may be removed by mechanical means or by use of overflow and recirculation tanks. This, however, is cumbersome and adds additional steps, as well as cost, to the electropolishing operation, so that the inhibition of the foam by the addition of a defoaming agent, is greatly to be preferred.

Referring now to the half tones which form the illustrative figures in the present application, FIG. I to FIG. III and FIG. VII are  $Fe_3O_4$  surfaced cathodes. The "before and after" pictures show that there is no zinc plating where such cathodes are used. In contrast, FIG. IV to FIG. VI and FIG. VIII to FIG. XXIV show that where the cathode surface does not contain  $Fe_3O_4$ , there is a considerable build-up of zinc on the cathode. The conditions under which electropolishing was carried out with these various cathodes will be shown in the specific examples which are included hereinafter.

In actual operation, an open tank is made of hot-rolled steel or heat treated steel, which tank serves as the cathode. For every ampere of current to be applied, 0.665 liter of an aqueous caustic soda solution, containing from 572 to 763 g./liter of caustic soda are placed in the cathode tank. This quantity of electrolyte gives a solution density not in excess of 2.5 amps./liter. The temperature of this solution is maintained within the range of 70 to 90° F. To this solution is added one of the defoaming agents disclosed above, in the amount of .2 g./liter. The size of the cathode tank is about 20-25 times that of the workpiece anode, i.e., for an anode workpiece having an area of 1 square foot, the cathode tank has an area of

20-25 square feet. The work piece of zinc or zinc alloy which is the anode is placed in the electrolyte solution and using a current of 200 amperes for each square foot of workpiece area, thereby giving a current density of 200 amperes/square foot, electropolishing is carried out for a period of about 4 minutes. At the expiration of this time, the workpiece is removed from the electrolyte and is found to have a smooth, bright, lustrous surface, free of pitting. Additionally, it is noted, that the cathode tank is completely free of any zinc plate or spongy deposit and there is little if any foam or froth in the electrolyte, thus showing the effectiveness of the defoaming agent as well as the cathode having a surface containing  $Fe_3O_4$  in preventing the plating of zinc.

In order that those skilled in the art may better understand the method of the present invention and the manner in which it may be practiced, the following specific examples are given.

In the following examples, unless otherwise specified, the electropolishing is carried out in a 2000 ml. glass beaker, equipped with cooling coils and a hot plate. A 6" x 12" sheet of heat treated steel is formed into a cylindrical cathode and placed into the beaker and 1700 ml. of electrolyte are added to the beaker. The effective volume of electrolyte contained within the cylindrical cathode is about 1115 ml. A 3/4" x 1" workpiece having a total surface area of about .01 square foot, is secured to a work bar which is lowered into the electrolyte. This workpiece is a zinc alloy known by the trade name Zamak-3 (trademark of The New Jersey Zinc Company) and having the following composition as specified in the 1957 ASTM Supplement, Part 2, page 115:

|           |                 |
|-----------|-----------------|
| Aluminum  | 3.9-4.3%.       |
| Magnesium | 0.03-0.06%.     |
| Copper    | 0.10% maximum.  |
| Iron      | 0.075% maximum. |
| Lead      | 0.005% maximum. |
| Cadmium   | 0.004% maximum. |
| Tin       | 0.002% maximum. |
| Zinc      | remainder.      |

During the electropolishing, the electrolyte is agitated by means of work bar agitation, the work bar having a two inch displacement/one second stroke. A source of D.C. current is connected to the workpiece and electropolishing is carried out for the desired length of time.

The following table, wherein are incorporated Examples 1 through 14, illustrates the effect of varying the electrolyte concentration. In these examples, the voltage range is 5.0-7.8 volts and the applied current is 2.5 amperes.

TABLE I

| Ex. | Bath No. | Com-position, grams/liter NaOH | Anode current density, amps./ft. <sup>2</sup> | Contact time, min. | Temp., ° F. | Remarks                                                  |
|-----|----------|--------------------------------|-----------------------------------------------|--------------------|-------------|----------------------------------------------------------|
| 1   | 33       | 25                             | 200                                           | 4                  | 73-75       | Light grey oxide coating, no cleaning or polishing.      |
| 2   | 34       | 50                             | 200                                           | 4                  | 73-75       | Dark grey, blue oxide coating, no cleaning or polishing. |
| 3   | 35       | 100                            | 200                                           | 4                  | 73-75       | Light grey oxide coating, no cleaning or polishing.      |
| 4   | 36       | 200                            | 200                                           | 4                  | 73-75       | Do.                                                      |
| 5   | 37       | 300                            | 200                                           | 4                  | 73-75       | Do.                                                      |
| 6   | 38       | 400                            | 200                                           | 4                  | 73-75       | Do.                                                      |
| 7   | 39       | 500                            | 200                                           | 4                  | 73-75       | Clean but not bright.                                    |
| 8   | 46B      | 550                            | 200                                           | 4                  | 73-75       | Clean and bright.                                        |
| 9   | 47B      | 600                            | 200                                           | 4                  | 73-75       | Clean and very bright.                                   |
| 10  | 60B      | 665                            | 200                                           | 4                  | 73-75       | Do.                                                      |
| 11  | 79A-2    | 800                            | 200                                           | 4                  | 110         | Clean but not bright, pitted.                            |
| 12  | 80A-2    | 903                            | 200                                           | 4                  | 121         | Do.                                                      |
| 13  | 81A-2    | 1,003                          | 200                                           | 4                  | 140         | Do.                                                      |
| 14  | 82A-2    | 1,190                          | 200                                           | 4                  | 149         | Do.                                                      |

<sup>1</sup> In Examples 11-14 it was necessary to increase the temperature to the value shown in order to put the desired amount of NaOH in solution.

As seen in the table, when the current density and temperature (except where indicated above) are kept constant, electropolishing does not take place until the composition of the electrolyte is about 450 g. of caustic soda/liter and that as the caustic soda concentration is increased, no polishing occurs above a concentration of 800 g./liter.

The following table incorporating Examples XV to XXIII, indicates the results obtained by varying the anode current density. In these examples, the voltage range is 6-11 volts and the contact time is 4 minutes.

TABLE II

| Ex.  | Bath No. | Composition, grams/liter NaOH | Anode current density, amps./ft. <sup>2</sup> | Applied current, amps. | Temp., °F.      | Remarks                       | 15 |
|------|----------|-------------------------------|-----------------------------------------------|------------------------|-----------------|-------------------------------|----|
| 15-- | 46A      | 550                           | 100                                           | 1.5                    | 73-75           | Clean but not bright.         | 24 |
|      | 46B      | 550                           | 200                                           | 2.5                    | 73-75           | Clean and bright.             | 25 |
|      | 46C      | 550                           | 400                                           | 4.5                    | 73-75           | Do.                           | 26 |
| 16-- | 47A      | 600                           | 100                                           | 1.5                    | 73-75           | Clean and very bright.        | 27 |
|      | 47B      | 600                           | 200                                           | 2.5                    | 73-75           | Do.                           | 28 |
| 17-- | 47C      | 600                           | 400                                           | 4.5                    | 73-75           | Clean and bright.             | 29 |
|      | 60A      | 665                           | 100                                           | 1.25                   | 73-75           | Clean and very bright.        | 30 |
|      | 60B      | 665                           | 200                                           | 2.5                    | 73-75           | Clean and very bright.        | 31 |
| 18-- | 60C      | 665                           | 400                                           | 5.0                    | 73-75           | Do.                           | 32 |
|      | 79A-1    | 800                           | 100                                           | 1.5                    | 99 <sup>1</sup> | Clean but not bright, pitted. | 33 |
| 19-- | 79A-2    | 800                           | 200                                           | 2.5                    | 110             | Do.                           | 34 |
|      | 79A-3    | 800                           | 400                                           | 4.5                    | 115             | Do.                           | 35 |
| 20-- | 80A-1    | 903                           | 100                                           | 1.5                    | 121             | Do.                           | 36 |
|      | 80A-2    | 903                           | 200                                           | 2.5                    | 121             | Do.                           | 37 |
|      | 80A-3    | 903                           | 400                                           | 4.5                    | 123             | Do.                           | 38 |
| 21-- | 81A-1    | 1,003                         | 100                                           | 1.5                    | 140             | Clean but not bright.         | 39 |
|      | 81A-2    | 1,003                         | 200                                           | 2.5                    | 140             | Do.                           | 40 |
|      | 81A-3    | 1,003                         | 400                                           | 4.5                    | 155             | Do.                           | 41 |
| 22-- | 82A-1    | 1,190                         | 100                                           | 1.5                    | 147             | Not clean or bright.          | 42 |
|      | 82A-2    | 1,190                         | 200                                           | 2.5                    | 149             | Clean but not bright.         | 43 |
|      | 82A-3    | 1,190                         | 400                                           | 4.5                    | 160             | Do.                           | 44 |
| 23-- | 84H-1    | 665                           | 600                                           | NM                     | 74              | Clean and very bright.        | 45 |
|      | 84H-2    | 665                           | 1000                                          | NM                     | 74              | Do.                           |    |
|      | 112A-4   | 665                           | 800                                           | NM                     | 74-75           | Do.                           |    |

<sup>1</sup> In Examples 18-21 it was necessary to increase the temperature to the value shown, in order to put the desired amount of NaOH in solution.

From this table, it is seen that when using current densities of less than 200 amps./square foot, no bright polishing occurs until the composition of the electrolyte is at least 600 g. of caustic soda/liter and that above this concentration, the polishing obtained when using 100 amps./square foot is not as good as that obtained when using a current density of 200 amps./square foot. Additionally, it can be seen that current densities greater than 200 amps./square foot do not produce results which are ap-

preciable superior to those obtained when using 200 amps./square foot, so that no advantage is obtained in using higher current densities.

In the following table, incorporating Examples 24-45, the effect of varying the temperature of the electrolyte can be seen. In these examples, the voltage is 4.8 volts, the applied current is 2.5 amperes, the anode current density is 200 amps./square foot and the contact time is 4 minutes.

TABLE III

| Ex. | Bath No. | Composition, grams/liter NaOH | Temp., °F. | Remarks                                   |
|-----|----------|-------------------------------|------------|-------------------------------------------|
| 24  | 84A-2    | 665                           | 76         | Clean and very bright.                    |
| 25  | 12B-2    | 665                           | 97-99      | Clean and bright.                         |
| 26  | 84B-2    | 665                           | 110        | Clean but not bright, light brown smut.   |
| 27  | 84C-2    | 665                           | 134        | Clean but not bright, light grey coating. |
| 28  | 84E-2    | 665                           | 152        | Light grey coating.                       |
| 29  | 84F-2    | 665                           | 180        | Dark grey coating.                        |
| 30  | 84G-2    | 665                           | 199        | Do.                                       |
| 31  | 79A-2    | 800                           | 110        | Clean but not bright, pitted.             |
| 32  | 79B-2    | 800                           | 129        | Clean and bright, slightly pitted.        |
| 33  | 79D-2    | 800                           | 154        | Dark grey oxide coating.                  |
| 34  | 79E-2    | 800                           | 178        | Do.                                       |
| 35  | 79F-2    | 800                           | 201        | Do.                                       |
| 36  | 80A-2    | 903                           | 121        | Clean and bright, pitting.                |
| 37  | 80B-2    | 903                           | 162        | Clean and bright, light brown film.       |
| 38  | 80C-2    | 903                           | 171        | Dark brown coating.                       |
| 39  | 80D-2    | 903                           | 203        | Dull bright grey oxide coating.           |
| 40  | 81A-2    | 1,003                         | 140        | Clean but not bright.                     |
| 41  | 81B-2    | 1,003                         | 174        | Dark grey oxide coating.                  |
| 42  | 81C-2    | 1,003                         | 206        | Do.                                       |
| 43  | 82A-2    | 1,190                         | 149        | Clean but not bright.                     |
| 44  | 82B-2    | 1,190                         | 179        | Clean but not bright, light grey smut.    |
| 45  | 82C-2    | 1,190                         | 198        | Dark grey coating.                        |

From this table it is seen that with electrolyte concentrations of 665 g. of caustic soda/liter, no brightening of the workpiece occurs at temperatures above 99° F., while no cleaning and smoothing occurs at temperatures in excess of 134° F. Likewise, at higher concentrations of caustic soda, there is some cleaning and brightening at higher temperatures, but even at these higher concentrations no brightening occurs above about 160° F. and there is no cleaning above about 180° F.

The following table, incorporating Examples 46-62, illustrates the effects obtained by incorporating zinc oxide and other metallic oxides in the caustic soda electrolyte composition. In these examples, the voltage range is 4.8-6.2 volts, the temperature varied between 73-75° F. and the contact time is 4 minutes.

TABLE IV

| Ex. | Bath No. | Composition, grams/liter |     |       | Anode current density, amps./ft. <sup>2</sup> | Applied current, amps. | Remarks                                                 |
|-----|----------|--------------------------|-----|-------|-----------------------------------------------|------------------------|---------------------------------------------------------|
|     |          | NaOH                     | ZnO | Other |                                               |                        |                                                         |
| 46  | 40       | 25                       | 10  | ----- | 200                                           | 2.5                    | Light grey oxide coating, no cleaning or polishing.     |
| 47  | 43A      | 50                       | 10  | ----- | 200                                           | 2.5                    | Dark grey-blue oxide coating, no cleaning or polishing. |
| 48  | 44A      | 75                       | 20  | ----- | 200                                           | 2.5                    | Do.                                                     |
| 49  | 41       | 100                      | 30  | ----- | 200                                           | 2.5                    | Do.                                                     |
| 50  | 45A      | 100                      | 50  | ----- | 200                                           | 2.5                    | Light grey oxide coating, no cleaning or polishing.     |
| 51  | 42       | 300                      | 50  | ----- | 200                                           | 2.5                    | Partial cleaning but no polishing.                      |
| 52  | 48A      | 400                      | 75  | ----- | 100                                           | 1.25                   | Do.                                                     |
|     | 48B      | 400                      | 75  | ----- | 200                                           | 2.5                    | Do.                                                     |
|     | 48C      | 400                      | 75  | ----- | 400                                           | 4.5                    | Do.                                                     |
| 53  | 49A      | 500                      | 25  | ----- | 100                                           | 1.25                   | Do.                                                     |
|     | 49B      | 500                      | 25  | ----- | 200                                           | 2.5                    | Do.                                                     |
|     | 49C      | 500                      | 25  | ----- | 400                                           | 4.5                    | Do.                                                     |
| 54  | 50A      | 500                      | 100 | ----- | 100                                           | 1.25                   | Cleaning and slight polishing.                          |
|     | 50B      | 500                      | 100 | ----- | 200                                           | 2.5                    | Do.                                                     |
|     | 50C      | 500                      | 100 | ----- | 400                                           | 4.5                    | Do.                                                     |
| 55  | 51A      | 600                      | 25  | ----- | 100                                           | 1.25                   | Clean and bright.                                       |
|     | 51B      | 600                      | 25  | ----- | 200                                           | 2.5                    | Do.                                                     |
|     | 51C      | 600                      | 25  | ----- | 400                                           | 4.5                    | Do.                                                     |
| 56  | 52A      | 600                      | 75  | ----- | 100                                           | 1.25                   | Do.                                                     |
|     | 52B      | 600                      | 75  | ----- | 200                                           | 2.5                    | Do.                                                     |
|     | 52C      | 600                      | 75  | ----- | 400                                           | 4.5                    | Do.                                                     |
| 57  | 53A      | 625                      | 25  | ----- | 100                                           | 1.25                   | Do.                                                     |
|     | 53B      | 625                      | 25  | ----- | 200                                           | 2.5                    | Clean and very bright.                                  |
|     | 53C      | 625                      | 25  | ----- | 400                                           | 4.5                    | Do.                                                     |
| 58  | 54A      | 665                      | 50  | ----- | 100                                           | 1.25                   | Clean and bright.                                       |
|     | 54B      | 665                      | 50  | ----- | 200                                           | 2.5                    | Clean and very bright.                                  |
|     | 54C      | 665                      | 50  | ----- | 400                                           | 4.5                    | Do.                                                     |

TABLE IV—Continued

| Ex.    | Bath No. | Composition, grams/liter |                                     |       | Anode current density, amps./ft. <sup>2</sup> | Applied current, amps.     | Remarks |
|--------|----------|--------------------------|-------------------------------------|-------|-----------------------------------------------|----------------------------|---------|
|        |          | NaOH                     | ZnO                                 | Other |                                               |                            |         |
| 59.... | 67A      | 665                      | Al <sub>2</sub> O <sub>3</sub> -100 | 100   | 1.25                                          | Clean but not bright.      |         |
|        | 67B      | 665                      | Al <sub>2</sub> O <sub>3</sub> -100 | 200   | 2.5                                           | Clean and bright.          |         |
|        | 67C      | 665                      | Al <sub>2</sub> O <sub>3</sub> -100 | 400   | 4.5                                           | Do.                        |         |
| 60.... | 68A      | 665                      | Al <sub>2</sub> O <sub>3</sub> -25  | 100   | 1.25                                          | Clean but not bright.      |         |
|        | 68B      | 665                      | Al <sub>2</sub> O <sub>3</sub> -25  | 200   | 2.5                                           | Clean and bright.          |         |
|        | 68C      | 665                      | Al <sub>2</sub> O <sub>3</sub> -25  | 400   | 4.5                                           | Do.                        |         |
| 61.... | 69A      | 665                      | MgO-25                              | 100   | 1.25                                          | Clean but not bright.      |         |
|        | 69B      | 665                      | MgO-25                              | 200   | 2.5                                           | Clean and bright.          |         |
|        | 69C      | 665                      | MgO-25                              | 400   | 4.5                                           | Do.                        |         |
| 62.... | 70A      | 665                      | MgO-2                               | 100   | 1.25                                          | Clean and slightly bright. |         |
|        | 70B      | 665                      | MgO-2                               | 200   | 2.5                                           | Clean and very bright.     |         |
|        | 70C      | 665                      | MgO-2                               | 400   | 4.5                                           | Do.                        |         |

By comparing the above results with those in Table I, it is seen that there is no appreciable difference between electropolishing with and without zinc oxide or some other oxide in the caustic soda electrolyte. In either case, electropolishing does not begin until the critical concentration of about 500 g. of caustic soda/liter is reached. Hence, although these oxides do not appear to adversely affect the electropolishing, their presence in the electrolyte is apparently superfluous.

The following table, incorporating Examples 63–67, shows the results obtained in determining the feasibility of carrying out electropolishing at a lower current density over a longer period of time. In these examples, the voltage range is 5.2–5.8 volts.

From the table, it is seen that no cleaning occurs until a current density of at least 40 amps./square foot is used and that no polishing occurs until a current density of at least 60 amps. per square foot is used, but in either instance, the time required is 45–60 minutes. Thus, although electropolishing can be carried out at current densities below that of the preferred 200 amps./square foot the time required for such an operation would not make it economically feasible and additionally larger equipment would be required.

| Ex.    | Bath No. | Applied current, amps. | Current density, amps./ft. <sup>2</sup> (as calculated from panels) | Remarks                                                     | TABLE VI                         |  |
|--------|----------|------------------------|---------------------------------------------------------------------|-------------------------------------------------------------|----------------------------------|--|
|        |          |                        |                                                                     |                                                             | 20                               |  |
| 68.... | 3202-A   | 0.1                    | .1-7                                                                | Grey dull surface over full current density range of panel. |                                  |  |
| 25     | 69....   | 3202-B                 | 0.5                                                                 | .5-25                                                       |                                  |  |
| 70.... | 3202-C   | 1                      | 1-4                                                                 | Do.                                                         |                                  |  |
|        |          |                        | 4-50                                                                | Grey dull surface.                                          |                                  |  |
| 71.... | 3202-D   | 2                      | 1-35                                                                | Brown oxide film with partial cleaning underneath.          |                                  |  |
|        |          |                        | 35-90                                                               | Do.                                                         |                                  |  |
| 30     | 72....   | 3202-E                 | 3                                                                   | 1-40                                                        | Clean and smooth but not bright. |  |
|        |          |                        | 40-150                                                              | Brown oxide film with partial cleaning underneath.          |                                  |  |
|        |          |                        | 150-170                                                             | Clean and smooth but not bright.                            |                                  |  |
| 73.... | 3202-F   | 5                      | 1-50                                                                | Clean and smooth, semi-bright.                              |                                  |  |
| 35     |          |                        | 50-175                                                              | Brown film, with partial cleaning underneath.               |                                  |  |
|        |          |                        | 175-300                                                             | Clean and smooth, semi-bright.                              |                                  |  |
| 74.... | 3202-II  | 10                     | 1-50                                                                | Very bright, electropolished.                               |                                  |  |
|        |          |                        | 50-180                                                              | Light brown film, clean underneath.                         |                                  |  |
|        |          |                        | 180-300                                                             | Clean and smooth, semi-bright.                              |                                  |  |
|        |          |                        |                                                                     | Very bright, electropolished.                               |                                  |  |

TABLE V

| Ex.    | Bath No. | Composition, grams/liter |     | Anode current density, amps./ft. <sup>2</sup> | Contact time, min. | Temp., °F. | Remarks                                       |
|--------|----------|--------------------------|-----|-----------------------------------------------|--------------------|------------|-----------------------------------------------|
|        |          | NaOH                     | ZnO |                                               |                    |            |                                               |
| 63.... | 120A-1   | 665                      | 100 | 10                                            | 5                  | 75         | Grey oxide coating, no cleaning or polishing. |
|        | 120A-2   | 665                      | 100 | 10                                            | 15                 | 75         | Do.                                           |
|        | 120A-3   | 665                      | 100 | 10                                            | 30                 | 75         | Do.                                           |
|        | 120A-4   | 665                      | 100 | 10                                            | 45                 | 75         | Do.                                           |
| 64.... | 120B-1   | 665                      | 100 | 20                                            | 5                  | 76         | Do.                                           |
|        | 120B-2   | 665                      | 100 | 20                                            | 15                 | 76         | Do.                                           |
|        | 120B-3   | 665                      | 100 | 20                                            | 30                 | 76         | Do.                                           |
|        | 120B-4   | 665                      | 100 | 20                                            | 45                 | 76         | Do.                                           |
| 65.... | 120C-1   | 665                      | 100 | 40                                            | 5                  | 78         | Clean but not polished.                       |
|        | 120C-2   | 665                      | 100 | 40                                            | 15                 | 78         | Do.                                           |
|        | 120C-3   | 665                      | 100 | 40                                            | 30                 | 78         | Do.                                           |
|        | 120C-4   | 665                      | 100 | 40                                            | 45                 | 78         | Do.                                           |
| 66.... | 120D-1   | 665                      | 100 | 60                                            | 5                  | 81         | Do.                                           |
|        | 120D-2   | 665                      | 100 | 60                                            | 15                 | 81         | Clean and slightly polished.                  |
|        | 120D-3   | 665                      | 100 | 60                                            | 30                 | 81         | Do.                                           |
|        | 120D-4   | 665                      | 100 | 60                                            | 45                 | 81         | Clean and bright.                             |
| 67.... | 120E-1   | 665                      | 100 | 100                                           | 5                  | 82         | Clean but not polished.                       |
|        | 120E-2   | 665                      | 100 | 100                                           | 15                 | 82         | Clean and slightly polished.                  |
|        | 120E-3   | 665                      | 100 | 100                                           | 30                 | 82         | Clean and bright.                             |
|        | 120E-4   | 665                      | 100 | 100                                           | 45                 | 82         | Clean and very bright.                        |

The results in the following table, incorporating Examples 68–74, were obtained using a Hull cell. 267 ml. of electrolyte, containing 670 g. of sodium hydroxide/liter and 93 g. zinc oxide/liter are placed in the Hull cell and electropolishing carried out for a period of 4 minutes at each of the applied currents indicated. The temperature of the electrolyte varied between 68 and 92° F. The panels used are 2½" x 4" pure zinc sheets.

The above results indicate that pure zinc as well as zinc alloys can be electropolished by the method of the present invention. Additionally, the above results serve as a check on the results obtained in previous tables, indicating that a current density of about 50 amps./square foot is the critical point at which electropolishing begins 70 to take place.

## Example 75

To illustrate the build-up of zinc oxide concentration during electropolishing, a life test is made using as the electrolyte 5 liters of caustic soda solution in a hard rubber tank containing 668 g. of caustic soda/liter and 0.2 g./liter polyoxyethylene ester of mixed fatty and rosin acid (Renex 20) as a defoamer. During this test the anode current density is 200 amps./square foot, the cathode current density is 13.8 amps./square foot and the solution density is 1.6 amps./liter. The anodes used are  $\frac{1}{2}$  inch strips of Zamak-3 alloy having a total surface area of .04/square foot, while the cathode is two sheets, 7 inches x 7 inches of heat-treated iron having a surface area of 0.58/square foot. The temperature of the electrolyte is maintained within the range of about 75-95° F., the average temperature being about 80° F. The anode is electropolished continuously until it is about 75% consumed whereupon it is replaced with a new anode. The following table is a summary of

oxide, electropolishing is carried out in 31.5 liters of electrolyte containing 665 g. of sodium hydroxide/liter, 100 g. of zinc oxide/liter, 0.2 g. of defoaming agent/liter (Renex 20). The anode current density is 200 amps./square foot, the cathode current density 7.4 amps./square foot and the solution density is 1.27 amps./liter. The electropolishing is carried out in a 32 liter tank of heat-treated steel, which tank forms the cathode and has a surface area of 5.4 square foot. As the anode, 2 strips of Zamak-3 are used, having a total surface area of .20 square foot. As in Example 75, the anodes are electropolished until they are about 75% consumed whereupon they are replaced. The conditions of operation and results obtained are reported below in a tabular summary, the results being reported every 10-20 hours. It should be noted that observations made during the intervals between the reported data indicate no significant deviation from the general trend.

TABLE VIII

| Bath No. | Cumulative |              |         | Analysis, g./l. |       | Anode loss of Zn in grams, Cu-mulative | Anode efficiency, percent | Remarks                                                          |
|----------|------------|--------------|---------|-----------------|-------|----------------------------------------|---------------------------|------------------------------------------------------------------|
|          | Hrs.       | Amp. hrs./l. | Ft.²/l. | Free NaOH       | Zinc  |                                        |                           |                                                                  |
| 86-----  | 0.7        | .86          | .06     | 596             | 101.8 | 17.5                                   | 53                        | Anode clean, smooth and lustrous.                                |
|          | 21.2       | 26.8         | 2.0     | 585             | 108   | 450.0                                  | 40                        | Do.                                                              |
|          | 45.1       | 57.3         | 4.3     | 548             | 120   | 958.0                                  | 42                        | Do.                                                              |
|          | 68.3       | 87.0         | 6.45    | 509             | 137   | 1427.0                                 | 47                        | Do.                                                              |
|          | 84.0       | 106.0        | 7.68    | 428             | 153   | 1,746.5                                | 44                        | Do.                                                              |
|          | 98.8       | 125          | 9.29    | 477             | 160   | 2,038.0                                | 40                        | Do.                                                              |
|          | 114.8      | 143          | 10.61   | 484             | 177   | 2,280.5                                | 29                        | Do.                                                              |
|          | 122.0      | 150          | 11.11   | 508             | 173   | 2,367.0                                | 28                        | Remove 1.5 l. of bath and replace with 1.5 l. of 665 g./l. NaOH. |
|          | 131.2      | 160          | 11.85   | 512             | 180   | 2,461.5                                | 29                        | Anode clean, smooth and lustrous.                                |
|          | 164.4      | 185          | 13.8    | 473             | 188   | 2,766.5                                | 31                        | Do.                                                              |
|          | 176.9      | 215          | 15.9    | 472             | 190   | 3,201.0                                | 39                        | Anode clean, smooth and semibright.                              |
|          | 198.9      | 245          | 18.2    | 388             | 195   | 3,548.0                                | 34                        | Do.                                                              |
|          | 215.3      | 266          | 19.7    | 392             | 202   | 3,817.0                                | 32                        | Anode clean, smooth and not bright.                              |
|          | 236.9      | 294          | 21.8    | 388             | 212   | 4,153.5                                | 29                        | Do.                                                              |

operating conditions and results obtained over a run of about 740 hours. These results are reported as taken every 24-40 hours. It should be noted that observations made during the intervals between the reported data indicate no significant deviation from the general trend. It should be further noted that when the solution has reached the fourth cycle, the anode efficiencies are dropping rapidly.

By comparing the results of Example 76 with those in Example 75, it is seen, that as would be expected, the time required for the zinc oxide content of the electrolyte to build-up to the toleration point is about half again as long in the bath which does not contain zinc oxide as compared to that which does contain zinc oxide in the amount of 100 g./liter.

TABLE VII

| Bath No. | Cumulative |              |         | Analysis, g./l. |      | Anode loss of Zn in grams, cumulative | Anode Efficiency, percent | Remarks                                                                                    |
|----------|------------|--------------|---------|-----------------|------|---------------------------------------|---------------------------|--------------------------------------------------------------------------------------------|
|          | Hrs.       | Amp. hrs./l. | Ft.²/l. | Free NaOH       | Zinc |                                       |                           |                                                                                            |
| 29-----  | 8.5        | 13.6         | 1.02    | 657             | 23.4 | 41.2                                  | 50                        | Anode clean, smooth and bright.                                                            |
|          | 30.3       | 44.4         | 3.62    | 622             | 41.2 | 141.5                                 | 50                        | Do.                                                                                        |
|          | 62.5       | 100          | 7.4     | 596             | 63.2 | 302.5                                 | 49                        | Do.                                                                                        |
|          | 93.5       | 149          | 11.2    | 533             | 105  | 451.5                                 | 59                        | Do.                                                                                        |
|          | 125.8      | 201          | 15.1    | 522             | 125  | 586.0                                 | 42                        | Do.                                                                                        |
|          | 158.3      | 253          | 18.0    | 489             | 152  | 718.0                                 | 46                        | Anode clean and bright.                                                                    |
|          | 189.8      | 303          | 22.8    | 465             | 177  | 848.0                                 | 40                        | Do.                                                                                        |
|          | 216.7      | 348          | 26.2    | 439             | 193  | 926.5                                 | 24                        | Anode clean and semibright.                                                                |
|          | 255.1      | 409          | 30.8    | 425             | 204  | 1,017.5                               | 32                        | Removed 25% (by volume) of the bath and replaced with 1.25 l. of 670 g./l. NaOH.           |
|          | 262.8      | 421          | 31.6    | 476             | 155  | 1,047.0                               | 40                        | Anode clean, smooth and bright.                                                            |
|          | 291.3      | 467          | 35.1    | 425             | 175  | 1,150.5                               | 33                        | Do.                                                                                        |
|          | 302.2      | 484          | 36.4    | 436             | 198  | 1,187.5                               | 44                        | Removed 25% of bath and replaced with 1.25 l. of 670 g./l. NaOH.                           |
|          | 307.9      | 493          | 37.0    | 508             | 141  | 1,208.5                               | 44                        | Anode clean, smooth and bright.                                                            |
|          | 338.6      | 643          | 40.8    | 496             | 172  | 1,313.0                               | 35                        | Do.                                                                                        |
|          | 366.9      | 582          | 43.7    | 448             | 186  | 1,395.0                               | 33                        | Anode clean, smooth and semibright.                                                        |
|          | 348.3      | 626          | 47.0    | 388             | 204  | 1,490.0                               | 36                        | Do.                                                                                        |
|          | 428.2      | 668          | 50.2    | 368             | 212  | 1,558.0                               | 25                        | Anode clean, blue-black oxide coated. Replenished 40% of bath with 2 l. of 670 g./l. NaOH. |
|          | 527        | 737          | 55.2    | 437             | 156  | 1,716.7                               | 37                        | Anode clean, smooth and bright.                                                            |
|          | 567        | 793          | 59.6    | 382             | 171  | 1,824.5                               | 32                        | Do.                                                                                        |
|          | 608        | 851          | 64.2    | 362             | 185  | 1,918.2                               | 25                        | Anode clean, smooth and semibright.                                                        |
|          | 681        | 953          | 71.6    | 362             | 202  | 2,028.6                               | 12                        | Anode clean, smooth and not bright.                                                        |
|          | 736        | 1,029        | 77.2    | 320             | 212  | 2,082.0                               | 7.2                       | Anode clean but dull, oxide coated.                                                        |

Example 76

In order to show the zinc oxide build-up during electropolishing in an electrolyte which initially contains zinc

Example 77

To show the effect of daily replenishment of electrolyte to simulate drag-out with regard to the zinc oxide build-

up, a life test is made using 5 liters of electrolyte containing 669.8 g. of sodium hydroxide/liter, 93.6 g. of zinc oxide/liter and 0.2 g./liter defoamer (Renex 20). The anode current density is 200 amps./square foot, the cathode current density 13.8 amps./square foot and the solution density is 1.6 amps./liter. The temperature is maintained within the range of about 70-90° F. with the average temperature being about 80° F. The cathode is formed from two 7 inch x 7 inch sheets of heat-treated steel having a total surface area of .58 square foot. The anode is a 1/2 inch strip of Zamak-3 alloy having a total surface area of .04 square foot. 5% or 250 ml. of the electrolyte is removed daily and replenished with a like amount of fresh caustic solution (670 g. NaOH/liter). As in the two previous examples, the anode is electropolished until it is about 75% consumed, whereupon it is replaced. The operating conditions and results obtained over a period of about 700 hours are shown below in a tubular summary. It should be noted that observations made during

replacing it with fresh caustic soda (670 g./liter), even though containing about 95 g./liter of zinc oxide at the beginning, at the expiration of 700 hours' operation the zinc oxide concentration is still considerably below the toleration point. Examination of the anodes for the run and the various test specimen done at intervals show a clear, smooth and very lustrous zinc surface. Even at 700 hours, it is still electropolishing satisfactory.

The following examples show the results obtained in testing different materials as cathodes for use in the present process. The half-tones which form the illustrative figures of the present invention were made of the cathode before and after electropolishing. In all of these examples, electropolishing is carried out in a one liter beaker containing 784 ml. of electrolyte, containing 632 g./liter sodium hydroxide and 101 g./liter zinc oxide. The anode is of Zamak-3 and has an area of 0.052 square foot. The anode current density is 200 amps./square foot and the solution density is 1.

TABLE X

| Ex. | Cathode material                            | Cathode area, ft. <sup>2</sup> | Voltage average | Temp. average, ° F. | Current efficiency, percent | Remarks                                                                                 |
|-----|---------------------------------------------|--------------------------------|-----------------|---------------------|-----------------------------|-----------------------------------------------------------------------------------------|
| 78  | Drum steel, heat-treated                    | 0.156                          | 5.0             | 83                  | 47                          | No plating of Zn, H <sub>2</sub> gassing at cathode, very bright polish on anode.       |
| 79  | Stainless steel, heat treated               | 0.163                          | 5.0             | 78                  | 46.4                        | Do.                                                                                     |
| 80  | Magnetite                                   | 0.095                          | 4.7             | 84                  | 50.4                        | Do.                                                                                     |
| 81  | Cast iron, HCl cleaned                      | 0.073                          | 4.2             | 80                  | 55.2                        | Do.                                                                                     |
| 82  | Drum steel                                  | 0.156                          | 4.8             | 84                  | 54.2                        | Zn plate on cathode, no H <sub>2</sub> gassing at cathode, very bright polish on anode. |
| 83  | Stainless steel                             | 0.196                          | 5.0             | 82                  | 46                          | Do.                                                                                     |
| 84  | Fe <sub>3</sub> O <sub>4</sub> coated steel | 0.156                          | 5.2             | 82                  | 50.3                        | Do.                                                                                     |
| 85  | Pure zinc                                   | 0.156                          | 4.9             | 86                  | 0                           | Do.                                                                                     |
| 86  | Graphite                                    | 0.196                          | 5.0             | 82                  | 45.6                        | Do.                                                                                     |
| 87  | Galvanized steel                            | 0.156                          | 4.8             | 82                  | 51.6                        | Do.                                                                                     |
| 88  | Zamak-3                                     | 0.136                          | 4.8             | 80                  | 48.7                        | Do.                                                                                     |
| 89  | Nickel                                      | 0.226                          | 4.6             | 82                  | 53.1                        | Do.                                                                                     |
| 90  | Lead                                        | 0.198                          | 5.0             | 80                  | 47.8                        | Do.                                                                                     |
| 91  | Copper                                      | 0.153                          | 5.0             | 83                  | 49.4                        | Do.                                                                                     |
| 92  | Tungsten                                    | 0.087                          | 5.0             | 80                  | 50.2                        | Do.                                                                                     |
| 93  | Lead oxidized                               | 0.198                          | 4.6             | 80                  | 50.3                        | Do.                                                                                     |
| 94  | Copper oxidized                             | 0.153                          | 5.0             | 84                  | 49.1                        | Do.                                                                                     |
| 95  | Tungsten oxidized                           | 0.085                          | 2.5             | 76                  | 68.4                        | Do.                                                                                     |
| 96  | Platinum                                    | 0.045                          | 6.0             | 80                  | 49.4                        | Do.                                                                                     |
| 97  | Titanium                                    | 0.181                          | 4.9             | 79                  | 48.7                        | Do.                                                                                     |
| 98  | Zirconium                                   | 0.068                          | 5.4             | 89                  | 48.3                        | Do.                                                                                     |
| 99  | Silver                                      | 0.136                          | 5.0             | 81                  | 50.2                        | Do.                                                                                     |
| 100 | Molybdenum                                  | 0.068                          | 5.0             | 79                  | 51.3                        | Do.                                                                                     |
| 101 | Aluminum                                    | 0.198                          | 4.8             | 81                  | 50.6                        | Do.                                                                                     |
| 102 | Nickel plated copper                        | 0.138                          | 4.2             | 77                  | 51.2                        | Do.                                                                                     |
| 103 | Chromium plated copper                      | 0.138                          | 4.1             | 78                  | 45.3                        | Do.                                                                                     |

<sup>1</sup> Not measured.

the intervals between the reported data indicate no significant change from the general trend.

TABLE IX

| Bath No. | Cumulative |              | Analysis, g./l.      |           | Anode loss of Zn in grams cumulative | Anode efficiency, percent |      |
|----------|------------|--------------|----------------------|-----------|--------------------------------------|---------------------------|------|
|          | Hours      | Amp. hrs./l. | Ft. <sup>2</sup> /l. | Free NaOH | ZnO                                  |                           |      |
| 108      | 6          | 9.4          | 0.7                  | 621       | 95.6                                 | 33                        | 52.5 |
|          | 21         | 34           | 2.55                 | 580       | 106                                  | 91                        | 62   |
|          | 36         | 57           | 4.27                 | 149       | 103                                  | 1.0                       | 42   |
|          | 50         | 77           | 5.90                 | 556       | 105                                  | 208                       | 43   |
|          | 72         | 114          | 8.56                 | 533       | 117                                  | 294                       | 43   |
|          | 106        | 170          | 12.80                | 540       | 125                                  | 427                       | 40   |
|          | 128        | 213          | 15.80                | 544       | 122                                  | 522                       | 48   |
|          | 143        | 234          | 17.50                | 544       | 125                                  | 580                       | 50   |
|          | 176        | 279          | 20.90                | 528       | 124                                  | 698                       | 42   |
|          | 190        | 199          | 22.4                 | 533       | 122                                  | 753                       | 49   |
|          | 244        | 352          | 26.4                 | 475       | 117                                  | 881                       | 43   |
|          | 301        | 422          | 31.6                 | 120       | 1,101                                | 1,101                     | 45   |
|          | 357        | 500          | 37.6                 | 476       | 119                                  | 1,303                     | 43   |
|          | 422        | 591          | 44.4                 | 470       | 121                                  | 1,550                     | 44   |
|          | 486        | 681          | 51.2                 | 472       | 124                                  | 1,788                     | 44   |
|          | 536        | 751          | 56.4                 | 484       | 129                                  | 1,973                     | 41   |
|          | 619        | 867          | 65.0                 | 476       | 124                                  | 2,273                     | 43   |
|          | 679        | 950          | 71.2                 | 485       | 124                                  | 2,505                     | 44   |

From the above, it is seen that where the electrolyte is replenished daily by removing about 5% of its volume and

55 From the above, it is seen that only when the cathode has a surface which contains Fe<sub>3</sub>O<sub>4</sub> is there no plating of zinc on the cathode. With all of the other materials used, zinc plates on the cathode, and there is no evolution of hydrogen gas at the cathode.

In substantiating the visual observation of the above examples with experimental data, the following examples, 60 which are carried out separately, are given in which the oxygen and hydrogen efficiencies during electropolishing using various cathode materials are measured. In these examples, the anode is Zamak-3 and has an area of 0.65 square inch. The anode current density is 200 amps./square foot. The electrolyte is 750 ml. containing 632 g. sodium hydroxide/liter and 101 g. zinc oxide/liter. The applied current is 1 amp. and the solution density is 1.25 amps./liter.

70 From the table it can be seen that when using the cathode having a surface which contains Fe<sub>3</sub>O<sub>4</sub>, on which cathode there is no plating of zinc, the hydrogen current efficiencies are very high showing that in these instances electrolysis of the water in the electrolyte is taking place rather than plating of the zinc on the cathode.

TABLE XI

| Ex. | Cathode material                   | Cathode area inches <sup>2</sup> | Time min. | Volt. ave. | Temp. ave., F | Anode efficiency (weight loss), percent | O <sub>2</sub> Gas efficiency, percent | H <sub>2</sub> Gas efficiency, percent | Remarks                     |
|-----|------------------------------------|----------------------------------|-----------|------------|---------------|-----------------------------------------|----------------------------------------|----------------------------------------|-----------------------------|
| 104 | Drum steel.....                    | 18                               | 240       | 4.25       | 84            | 59.6                                    | 33.1                                   | 1.3                                    | Spongy Zn plated on cathode |
| 105 | 10/10 steel, pickled.....          | 15.3                             | 240       | 5.7        | 76            | 53.0                                    | 48.5                                   | 2.6                                    | Do.                         |
| 106 | Graphite.....                      | 9                                | 117       | 5.3        | 78            | 62.8                                    | 41.1                                   | 6.6                                    | Do.                         |
| 107 | Zirconium.....                     | 11                               | 151       | 5.4        | 81            | 67.1                                    | 48.3                                   | 12.6                                   | Do.                         |
| 108 | Stainless steel.....               | 15.9                             | 180       | 5.2        | 82            | 66.5                                    | 34                                     | 15                                     | Do.                         |
| 109 | Copper, oxidized.....              | 18                               | 89        | 5.8        | 78            | 70.4                                    | 33.3                                   | 15.2                                   | Do.                         |
| 110 | Nickel.....                        | 16.5                             | 172       | 5.2        | 81            | 71.0                                    | 36.1                                   | 18                                     | Do.                         |
| 111 | Molybdenum.....                    | 11.4                             | 150       | 6.2        | 76            | 65.7                                    | 40.5                                   | 24.4                                   | Do.                         |
| 112 | Cast iron, pickled.....            | 9.4                              | 203       | 5.6        | 76            | 58.4                                    | 36                                     | 52.5                                   | No Zn plate on cathode.     |
| 113 | Drum steel, heat treated.....      | 18                               | 188       | 5.4        | 82            | 50.2                                    | 45.1                                   | 81.2                                   | Do.                         |
| 114 | Stainless steel, heat treated..... | 11.3                             | 133       | 5.5        | 75            | 48.8                                    | 45.5                                   | 87.5                                   | Do.                         |

To attempt to explain the behavior of cathodes having a surface of  $Fe_3O_4$ , potential measurements are carried out with several cathode materials in both 45% caustic soda solution and sodium zincate (665 g./liter  $NaOH$ , 100 g./liter  $ZnO$ ) media. The measurements are made using the conventional "direct method" for electrode potential and over potentials under continuous electrolysis in a 1000 ml. solution with constant stirring.

Both the reference and the electropolishing cells are kept at a constant temperature of  $25^\circ\text{ C.} \pm 0.1$ . The anode area is kept constant at  $3.9\text{ cm.}^2$  while the cathode area varies from  $50\text{--}100\text{ cm.}^2$ . The anode material is Zamak-3 alloy. Because of the alkali medium, the reference electrode selected is mercury-mercuric oxide; it is checked with a standard saturated calomel electrode (0.2415 v.).

Table XII-A gives the reference electrode potentials for various sodium hydroxide concentrations. The values (unknown in literature) are reported to serve as the basis for the measurements. The E.M.F. of the mercury-mercuric oxide electrode with the zincate solution is determined to be 0.065 v. (not included in Table XII-A).

Table XII-B gives the values obtained with various cathodes under various current densities in both the 45% caustic soda and zincate media. FIGS. 25 and 26 give a graphic comparison of these potentials.

TABLE XII-A

## *Potentials of the Reference Electrode With Different Concentrations Alkali*

| NaHO<br>(Normality) | Average potential<br>HgHgO <sub>x</sub> NaOH<br>vs. S.C.E. | Average potential<br>of HgHgO Elec-<br>trode |
|---------------------|------------------------------------------------------------|----------------------------------------------|
| 0.97                | +0.1280                                                    | -0.1135                                      |
| 2.58                | +0.1429                                                    | -0.0986                                      |
| 5.34                | +0.1556                                                    | -0.0859                                      |
| 7.81                | +0.1662                                                    | -0.0753                                      |
| 10.30               | +0.1749                                                    | -0.0666                                      |
| 15.50               | +0.1892                                                    | -0.0524                                      |
| 17.50               | +0.1906                                                    | -0.0505                                      |
| 19.10               | +0.1895                                                    | -0.0531                                      |

TABLE XII-B

rent density (Table II) and the Hull cell test panel (Table VI).

While there have been described various embodiments of the invention, the methods described are not intended to be understood as limiting the scope of the invention, and it is realized that changes therewithin are possible, and it is further intended that each element recited in any of the following claims is to be understood as referring to all equivalent elements for accomplishing substantially the same results in substantially the same or equivalent manner, it being intended to cover the invention broadly in whatever form its principle may be utilized.

What is claimed is:

1. A method of anodically electropolishing an article having a surface of metal selected from the group consisting of zinc and zinc base alloys, which comprises making the article to be polished the anode in an electrolytic cell, the electrolyte of which is comprised of an alkali metal hydroxide in the amount between about 450 and 900 grams/liter, maintained at a temperature between about 60° and 220° F. and passing an electric current through said electrolyte between said anode and a cathode having a surface of  $Fe_3O_4$ , said current being passed at an anode current density between about 50 and 800 amps./square foot for a period of time sufficient to electropolish said anode, and using a voltage sufficient to provide this current density, said voltage being below that at which zinc will be electrodeposited on said cathode having a surface of  $Fe_3O_4$ .

2. A method of anodically electropolishing an article having a surface of metal selected from the group consisting of zinc and zinc base alloys, which comprises making the article to be polished the anode in an electrolytic cell, the electrolyte of which is comprised of an alkali metal hydroxide in the amount between 572 and 763 grams/liter, maintaining said electrolyte at a temperature between about 70° and 90° F., passing an electric current through said electrolyte between said anode and a cathode at an anode current density of about 200 amps./square foot, said cathode having a surface of  $Fe_3O_4$ , the passage of current being for a period of time sufficient to electropolish said anode, and using a voltage sufficient to provide the above current density, said voltage being below that at which zinc will be electrodeposited on said cathode having a surface of  $Fe_3O_4$ .

3. The method as claimed in claim 2, wherein the alkali metal hydroxide in the electrolyte is sodium hydroxide.

4. The method as claimed in claim 3, wherein the solution current density used does not exceed 2.5 amps./liter.

5. The method as claimed in claim 3, wherein the electrolyte contains zinc oxide in an amount up to about 175 grams/liter.

6. The method as claimed in claim 3, wherein a defoaming agent is added to the electrolyte.

7. The method as claimed in claim 5, wherein a defoaming agent is added to the electrolyte.

8. A method of anodically electropolishing an article having a surface of metal selected from the group consisting of zinc and zinc base alloys, which comprises making the article to be polished the anode in an electrolytic cell, the electrolyte of which is comprised of sodium hydroxide in the amount of about 665 grams/liter, maintained at a temperature of about 76° F. and passing an electric current through said electrolyte between said anode and a cathode at an anode current density of about 200 amps./square foot, said cathode having a surface of  $Fe_3O_4$ , the passage of current being for a period of time sufficient to electropolish said anode, and using a voltage sufficient to provide the above current density, said voltage being below that at which zinc will be electrodeposited on said cathode having a surface of  $Fe_3O_4$ .

9. The method as claimed in claim 7, wherein the electrolyte contains zinc oxide in an amount up to about 100 grams/liter.

10. The method as claimed in claim 8, wherein a defoaming agent is added to the electrolyte.

11. The method as claimed in claim 9, wherein a defoaming agent is added to the electrolyte.

12. The method as claimed in claim 8, wherein the solution current density is maintained below 2.5 amps./liter.

13. The method as claimed in claim 1, wherein the cathode is made of hot rolled steel.

14. The method as claimed in claim 2, wherein the cathode is made of hot rolled steel.

15. The method as claimed in claim 8, wherein the cathode is made of hot rolled steel.

#### References Cited in the file of this patent

#### UNITED STATES PATENTS

|           |           |       |               |
|-----------|-----------|-------|---------------|
| 670,201   | Kendall   | ----- | Mar. 19, 1901 |
| 931,513   | Specketer | ----- | Aug. 17, 1909 |
| 2,655,472 | Hilliard  | ----- | Oct. 13, 1953 |

#### OTHER REFERENCES

Nature, vol. 142, 1938, pp. 477-8, 1161.

Chemical Abstracts, 1942, vol. 36, p. 6919.

Canadian Journal of Chemistry, vol. 31, 1953, pp.

422-438.

UNITED STATES PATENT OFFICE  
CERTIFICATE OF CORRECTION

May 7, 1963

Patent No. 3,088,886

Joseph Adrien M. Le Duc

It is hereby certified that error appears in the above numbered patent requiring correction and that the said Letters Patent should read as corrected below.

Column 4, line 22, for "mount" read -- amount --; column 7, TABLE II, third column, line 5 thereof, for "609" read -- 600 --; columns 11 and 12, TABLE VIII, second column, line 8 thereof, for "122.0" read -- 122.9 --; same TABLE VIII, ninth column, line 10 thereof, for "Do<sub>2</sub>" read -- Do. --; column 13, line 18, for "tubular" read -- tabular --; columns 15 and 16, TABLE XI, in the heading to column 6 thereof, for "Temp. ave., F" read -- Temp. ave., °F. --; column 15, TABLE XII-A, in the heading to column 1 thereof, for "NaOH" read -- NaOH --; column 16, line 56, for "result" read -- results --.

Signed and sealed this 10th day of December 1963

(SEAL)

Attest:

ERNEST W. SWIDER

Attesting Officer

EDWIN L. REYNOLDS

Acting Commissioner of Patents